

## UNITED STATES PATENT OFFICE

2,232,318

## PROCESS FOR IMPROVING THE DYEING PROPERTIES OF ARTIFICIAL FIBERS, FOILS, FILMS, RIBBONS, AND THE LIKE, AND PRODUCTS OBTAINED THEREFROM

Paul Esselmann, Wolfen, Kreis Bitterfeld, and Josef Düsing, Dessau, Germany, assignors, by mesne assignments, to Walther H. Duisberg, New York, N. Y.

No Drawing. Application August 4, 1938, Serial No. 223,012. In Germany August 4, 1937

9 Claims. (Cl. 260—13)

This invention relates to a process of producing artificial fibers, films, foils, ribbons and the like materials capable of being dyed by acid wool dyestuffs.

5 It has been proposed to spin artificial fibers, such as rayon or rayon staple fibers from a viscose solution to which have been added protein substances. In this process the protein is added to the spinning solution only shortly before the 10 spinning in order to avoid any substantial degradation of the protein molecule.

In order to fix the incorporated proteins it has further been proposed to condense the fibers with formaldehyde or to treat them subsequently with 15 an amine.

It appeared, however, that a complete fixation of the protein substances within the cellulosic fibers has not been achieved in this manner.

It is therefore an object of the present invention to provide a process by which artificial textile materials capable of being dyed fastly by acid wool dyestuffs may be obtained.

20 A further object of the invention is the provision of artificial fibers which can be dyed together with wool and in the same dyeing bath in uniform tints.

25 Still another object is the provision of artificial fibers, threads and the like textile materials, which consist of cellulose hydrate, cellulose acetate or a similar film- or fiber-forming polymer and which contain dispersed therein an addition of a basic artificial resin.

30 Further objects of the invention will become apparent from the following detailed specification.

In our copending application of even date Ser. No. 223,013, we have described a new type of resinous compositions which are obtained by reacting an organic amine on a protein substance, and jointly polymerizing the reaction product together with an arylisocyanate or an arylisothiocyanate.

35 As suitable starting materials for the polymerization described in more detail in the said copending application the following may be named as examples.

40 Suitable organic bases are, for instance, the alkyleneimines, such as ethylene-, propylene- and butylene-imines, N-propyl-ethyleneimine and N-benzylethylenimine.

45 Furthermore aliphatic and aromatic amines, such as methylamine, stearylamine and aniline may be employed.

50 Suitable protein substances are casein, albumen, gelatin, and the like materials.

As aryliso- and arylisothiocyanates there may be employed mainly the phenyl- and naphthylisocyanates as well as the phenyl- and naphthylisothiocyanates, benzylisocyanate, and related compounds.

5 The resinous compositions produced according to the process referred to above in the spinning solutions for artificial fibers or in the casting solutions for films, foils, ribbons and the like materials, products may be obtained which can be dyed easily by acid dyestuffs. The products have the further advantage that the dyeings with acid dyestuffs are exceedingly fast against light and washing and that they resemble the dyeings on 10 wool in all respects.

15 The resinous compositions may be added to the spinning solutions either in the form of the reaction mixture or they may be isolated beforehand and added to the spinning solutions as 20 powdery substances.

25 It is further possible to produce an emulsion of the resinous compositions by adding solvents thereof and to add this emulsion to the spinning solutions.

Surprisingly it has proved that the spinning 30 solutions are not affected at all by these additions and that the spinning or casting may be effected in exactly the same manner as has hitherto been usual. No difficulties arise at all from the addition of the synthetic resins.

Thus the synthetic resins may be added to viscose solutions, to cuprammonium spinning solutions or to cellulose acetate solutions.

The finished fibers have exactly the same properties from the point of view of the colorist as 35 wool. The fastness to light and washing of dyeings thereon with acid wool dyestuffs equals that of wool.

The following examples further serve to illustrate the invention:

Example 1.—500 grams of casein are added in successive small portions while stirring to 10 liters of an aqueous solution of 15 per cent strength of ethyleneimine. This mixture is allowed to stand for 24 hours, during which period 45 the casein enters into reaction with the ethyleneimine and becomes quickly dissolved. The solution is cooled and 3 kilos of phenylisocyanate are added thereto drop by drop while strongly stirring. The white emulsion first produced gradually solidifies to a fine powder which is insoluble in dilute acids and alkalies. The product contains 22 per cent of nitrogen. It may be added 50 to the spinning solution in the form of an emul- 55

sion produced by making it into a paste with warm cyclohexanol. The thread obtained on spinning is very similar to wool in respect of being dyed.

*Example 2.*—1 kilo of casein is stirred cautiously in small portions into 5 liters of an aqueous solution of 30 per cent strength of ethyleneimine, and the whole is allowed to stand overnight. The mixture is diluted with 2 liters of trichlorethylene and there are added gradually by drops while cooling and stirring 5 kilos of phenylisocyanate. The white emulsion thus obtained is suspended in 2 liters of cyclohexanol and the whole is heated for 1 hour at 70° C. 300 grams of this emulsion are added to 10 liters of viscose (cellulose content 7.9 per cent, alkali content 6.3 per cent), and the mixture is stirred until the animalizing agent has been uniformly distributed in the viscose. The viscose thus obtained, after filtration and subjection to a vacuum, is spun. The animalized fiber has a good affinity for acid wool dyestuffs.

*Example 3.*—150 grams of casein are mixed with 1 liter of ethyleneimine of 15 per cent strength and after 24 hours the mixture is diluted with 200 cc. of water. 300 cc. of this mixture (proportion of casein to ethyleneimine=1:3) are cooled with ice water and there are added gradually by drops 120 cc. of phenylisocyanate while stirring. The product is an almost transparent highly viscous solution which may be directly emulsified with viscose. The spun fibers have a character similar to that of wool.

*Example 4.*—300 grams of casein are added in small portions while stirring to 1 liter of ethyleneimine of 30 per cent strength. The solution is allowed to stand overnight and then filtered. To the filtrate 300 cc. of phenylisothiocyanate are added drop by drop. When this addition is complete, the whole is heated for 2 hours at 70° C. From the product thus obtained there is prepared an emulsion in cyclohexanol and this is added to viscose.

*Example 5.*—500 grams of casein are stirred into 3.3 liters of a solution of ethyleneimine of 15 per cent strength. After a short heating to 40° C. the whole is left standing for 24 hours at room temperature. The casein is then completely dissolved. To this mixture of casein and ethyleneimine there are gradually added while stirring 1 liter of phenylisocyanate by drops. The temperature of the reaction mixture must not rise above 40° C. The white reaction product is carefully filtered and well washed with hot water. The condensation product is insoluble in dilute acids and alkalies. It is soluble, for instance, in pyridine, aniline and meta-toluidine. If this solution is added to a spinning solution fibers of wool-like character are obtained.

60     What we claim is:

1. Artificial textile materials capable of being dyed by acid wool dyestuffs in the same manner as wool, comprising a polymer useful in forming an artificial textile material incapable per se of being dyed by acid dyes, and finely distributed therein the product of a joint polymerization of the reaction product of an alkyleneimine and a protein, with a compound selected from the group consisting of arylisocyanates and arylisothiocyanates.

2. Artificial textile materials capable of being dyed by acid wool dyestuffs in the same manner as wool, comprising cellulose hydrate, and finely distributed therein the product of a joint polymerization of the reaction product of an alkyleneimine and a protein, with a compound selected from the group consisting of arylisocyanates and arylisothiocyanates. 5

3. Artificial textile materials capable of being dyed by acid wool dyestuffs in the same manner 10 as wool, comprising cellulose acetate, and finely distributed therein the product of a joint polymerization of the reaction product of an alkyleneimine and a protein, with a compound selected from the group consisting of arylisocyanates and 15 arylisothiocyanates.

4. Artificial textile materials capable of being dyed by acid wool dyestuffs in the same manner 20 as wool, comprising cellulose hydrate, and finely distributed therein the product of a joint polymerization of the reaction product of an alkyleneimine and a protein, with phenylisocyanate.

5. Artificial textile materials capable of being dyed by acid wool dyestuffs in the same manner 25 as wool, comprising cellulose hydrate, and finely distributed therein the product of a joint polymerization of the reaction product of ethyleneimine and casein, with phenylisocyanate.

6. Artificial textile materials capable of being dyed by acid wool dyestuffs in the same manner 30 as wool, comprising cellulose hydrate, and finely distributed therein the product of a joint polymerization of the reaction product of ethyleneimine and casein, with phenylisothiocyanate.

7. A process of producing artificial textile materials capable of being dyed by acid wool dye-stuffs, which process comprises finely dispersing in the solution from which the said materials are to be formed, a synthetic resinous composition stable against dilute acids and alkalies, said resinous composition being the product of a joint polymerization of the reaction product of an alkyleneimine and a protein, with a compound selected from the group consisting of arylisocyanates and arylisothiocyanates. 35

8. A process of producing artificial textile materials capable of being dyed by acid wool dye-stuffs, which process comprises finely dispersing in the solution from which the said materials are to be formed, solid particles of a synthetic resinous composition stable against dilute acids and alkalies, said resinous composition being the product of a joint polymerization of the reaction product of an alkyleneimine and a protein, with a compound selected from the group consisting of arylisocyanates and arylisothiocyanates. 40

9. A process of producing artificial textile materials capable of being dyed by acid wool dye-stuffs, which process comprises finely dispersing in the solution from which the said materials are to be formed, a suspension in an organic solvent of a synthetic resinous composition stable against dilute acids and alkalies, said resinous composition being the product of a joint polymerization of the reaction product of an alkyleneimine with 65 a protein, and a compound selected from the group consisting of arylisocyanates and arylisothiocyanates.

PAUL ESSLEMANN.  
JOSEF DÜSING.

70